



US007545561B2

(12) **United States Patent**  
**Adachi et al.**

(10) **Patent No.:** **US 7,545,561 B2**  
(45) **Date of Patent:** **Jun. 9, 2009**

(54) **IMAGE DISPLAY AND METHOD FOR EVALUATING GLASS SUBSTRATE TO BE USED IN SAME**

(75) Inventors: **Daisuke Adachi**, Kameoka (JP); **Hiroyasu Tsuji**, Sennan-gun (JP); **Keisuke Sumida**, Hirakata (JP)

(73) Assignee: **Panasonic Corporation**, Osaka (JP)

(\*) Notice: Subject to any disclaimer, the term of this patent is extended or adjusted under 35 U.S.C. 154(b) by 680 days.

(21) Appl. No.: **10/499,339**

(22) PCT Filed: **Nov. 27, 2003**

(86) PCT No.: **PCT/JP03/15123**

§ 371 (c)(1),  
(2), (4) Date: **Jun. 17, 2004**

(87) PCT Pub. No.: **WO2004/051606**

PCT Pub. Date: **Jun. 17, 2004**

(65) **Prior Publication Data**

US 2005/0062416 A1 Mar. 24, 2005

(30) **Foreign Application Priority Data**

Nov. 29, 2002 (JP) ..... 2002-347188

(51) **Int. Cl.**

**G06K 7/10** (2006.01)

(52) **U.S. Cl.** ..... **359/350**; 359/900; 359/896;  
356/51; 356/445; 65/29.18

(58) **Field of Classification Search** ..... None  
See application file for complete search history.

(56) **References Cited**

U.S. PATENT DOCUMENTS

|                   |        |                    |          |
|-------------------|--------|--------------------|----------|
| 3,674,453 A *     | 7/1972 | Loukes et al. .... | 65/30.13 |
| 2002/0105721 A1 * | 8/2002 | Paul et al. ....   | 359/359  |
| 2005/0073475 A1 * | 4/2005 | Adachi et al. .... | 345/60   |
| 2007/0209394 A1 * | 9/2007 | Adachi et al. .... | 65/29.18 |

FOREIGN PATENT DOCUMENTS

|    |           |        |
|----|-----------|--------|
| JP | 60-107547 | 6/1985 |
| JP | 10-144208 | 5/1998 |
| JP | 10-255669 | 9/1998 |

(Continued)

OTHER PUBLICATIONS

NB78044795, 'Method to detect tin contamination on plate glass', IBM Technical Disclosure Bulletin, vol. 20, No. 11B, Apr. 1, 1978, pp. 4795-4796.\*

(Continued)

*Primary Examiner*—Arnel C Lavarias

(74) *Attorney, Agent, or Firm*—Wenderoth, Lind & Ponack, L.L.P.

(57) **ABSTRACT**

Provided are an image display device capable of displaying a good image by suppressing yellowing of a glass substrate, and an evaluating method of the glass substrate. The image display device is formed using the glass substrate where reflectance at wavelength of 220 nm is 5% or lower. In the evaluating method of the glass substrate for the image display device, Sn<sup>++</sup> content in the glass substrate is analyzed using reflectance at wavelength of 220 nm.

**1 Claim, 6 Drawing Sheets**



FOREIGN PATENT DOCUMENTS

|    |             |         |
|----|-------------|---------|
| JP | 11-67101    | 3/1999  |
| JP | 11-144623   | 5/1999  |
| JP | 11-246238   | 9/1999  |
| JP | 2000-169764 | 6/2000  |
| JP | 2002-298744 | 10/2002 |

JP 2002-324483 11/2002

OTHER PUBLICATIONS

“Glass Substrate PD200”, Asahi Glass Co. Ltd., 2001 FPD Technology Outlook pp. 706-707.

\* cited by examiner

FIG. 1



FIG. 2



FIG. 3



FIG. 4



FIG. 5



FIG. 6



FIG. 7



FIG. 8



FIG. 9



## 1

**IMAGE DISPLAY AND METHOD FOR  
EVALUATING GLASS SUBSTRATE TO BE  
USED IN SAME**

TECHNICAL FIELD

The present invention relates to an image display device such as a plasma display panel (PDP) and an evaluating method of a glass substrate for use in it.

BACKGROUND ART

There are various types of image display devices for displaying a high definition television image on a large screen. PDPs belong to one of the various types. A PDP is hereinafter described as an example.

A PDP is formed of two glass substrates: a front-side glass substrate for displaying an image; and a back-side glass substrate facing the front-side glass substrate. The front-side glass substrate has the following elements:

- a display electrode that is formed on one principal surface thereof and includes a stripe-like transparent electrode and a bus electrode;
  - a dielectric film that covers the display electrode and works as a capacitor; and
  - a MgO protective layer formed on the dielectric film.
- The back-side glass substrate has the following elements:
- a stripe-like address electrode formed on one principal surface thereof;
  - a dielectric film for covering the address electrode;
  - barrier ribs formed on the dielectric film; and
  - phosphor layers that are formed between the barrier ribs and emit red light, green light, and blue light, respectively.

As the front-side glass substrate and the back-side glass substrate, glass substrates that are easily increased in area, have high flatness, are inexpensive, and are manufactured by a float method are used. These glass substrates are disclosed in Electronic Journal, Separate Volume "2001, FPD Technology Summa" (Electronic Journal Co. Ltd. Oct. 25, 2000, p706-p707).

The float method is a method of forming plate-shaped glass by floating and conveying molten glass onto molten metallic tin under reducing atmosphere. An inexpensive glass sheet having large area can be precisely manufactured in the float method, so that the float method is in widespread use in manufacturing of a window glass or the like.

When an Ag electrode made of silver material is formed on a float glass substrate manufactured by the float method, however, a colored layer is disadvantageously formed on the surface of the glass substrate and the glass substrate changes into yellow (yellows).

This coloring phenomenon of the glass substrate by the Ag electrode is caused by the following processes:

- a silver colloid is generated by oxidation-reduction reaction between reducing bivalent tin ions ( $Sn^{++}$ ) existing on the glass substrate and silver ions ( $Ag^+$ ); and
- light absorption therefore occurs near wavelength of 350 to 450 nm.

In other words, the glass substrate is exposed to the reducing atmosphere containing hydrogen in a molding process in a float furnace as a molten metallic tin bath. A reducing layer with a thickness of several  $\mu m$  containing tin ions ( $Sn^{++}$ ) of the molten tin (Sn) is generated on the surface of the glass substrate. When a bus electrode including an Ag electrode is formed on the glass substrate having the reducing layer on its surface, silver ions ( $Ag^+$ ) separate from the bus electrode, and

## 2

infiltrate into the glass due to ion exchange with alkali metal ions contained in the glass. The infiltrating silver ions ( $Ag^+$ ) are reduced by the tin ions ( $Sn^{++}$ ) existing in the reducing layer to generate metallic silver (Ag) colloid. The metallic silver (Ag) colloid yellows the glass substrate. The yellowing also occurs on the front-side glass substrate having the bus electrode on the transparent electrode.

When the glass substrate, especially the front-side glass substrate, yellows, the yellowing is fatal in the image display device. Due to the yellowing of the glass substrate, the panel looks yellow, the commercial value decreases, display brightness of blue decreases to change display chromaticity, and color temperature decreases to degrade picture quality especially in displaying white.

These problems occur not only in a PDP but also in a general image display device having a structure where an Ag electrode is formed on a glass substrate.

The present invention addresses the problems, provides an image display device allowing good image display by suppressing yellowing of the glass substrate, and provides an evaluating method of the glass substrate for use in the image display device.

SUMMARY OF THE INVENTION

An image display device of the present invention, for addressing the problems, employs a glass substrate of which reflectance at a wavelength of 220 nm is 5% or lower.

Thanks to this structure, even in the image display device where an electrode made of Ag material is formed on the glass substrate manufactured by the float method, the glass substrate does not yellow and the image display quality is high.

In the evaluating method of the glass substrate for the image display device of the present invention, content of  $Sn^{++}$  in the glass substrate is analyzed based on the reflectance at wavelength of 220 nm. In providing an image display device by forming an electrode made of Ag material on a glass substrate manufactured by the float method, this evaluating method allows easy and efficient selection of a glass substrate that does not yellow and provision of a glass substrate optimum for an image display device having high image display quality.

BRIEF DESCRIPTION OF THE DRAWINGS

FIG. 1 is a sectional and perspective view showing a schematic structure of a PDP as an image display device in accordance with an exemplary embodiment of the present invention.

FIG. 2 is a graph showing a relation between a surface removing amount and a reflection spectrum of a glass substrate manufactured by a float method.

FIG. 3 is a graph showing a relation between reflectance at the wavelength of 220 nm and coloring degree of glass.

FIG. 4 is a graph showing difference  $\Delta R$  between reflection spectrum  $R_S(\lambda)$  of the glass substrate and reflection spectrum  $R_B(\lambda)$  in a nonexistent state of  $Sn^{++}$ .

FIG. 5 is a graph showing an analyzing result of the reflection spectrum of the glass substrate.

FIG. 6 is a graph illustrating wavelength  $\lambda^*$  maximizing difference  $\Delta R$  between reflection spectrum  $R_S(\lambda)$  of the glass substrate and reflection spectrum  $R_B(\lambda)$  in a nonexistent state of  $Sn^{++}$ .

FIG. 7 is a schematic block diagram of a manufacturing apparatus of the glass substrate for the image display device in accordance with the exemplary embodiment of the present invention.

FIG. 8 is a schematic block diagram of another manufacturing apparatus of the glass substrate for the image display device in accordance with the exemplary embodiment.

FIG. 9 is a schematic block diagram of still another manufacturing apparatus of the glass substrate for the image display device in accordance with the exemplary embodiment.

#### DETAILED DESCRIPTION OF PREFERRED EMBODIMENTS

An exemplary embodiment of the present invention will be described with reference to the drawings.

A PDP is hereinafter described as an example of image display devices. However, the present invention is useful for an image display device having a structure where an electrode made of Ag material is disposed on a glass substrate that is manufactured by the float method and has Sn<sup>++</sup> on its surface.

FIG. 1 is a sectional and perspective view showing a schematic structure of the PDP. PDP 1 is formed of two glass substrates: front-side glass substrate 3 for displaying an image; and back-side glass substrate 10 facing the front-side glass substrate.

Front substrate 2 of PDP 1 has the following elements: display electrodes 6 that are formed on one principal surface of front-side glass substrate 3 and include scan electrode 4 and sustain electrode 5; dielectric layer 7 for covering display electrodes 6; and protective layer 8, made of MgO for example, for covering dielectric layer 7.

In scan electrode 4 and sustain electrode 5, for decreasing electric resistance, bus electrodes 4b and 5b made of Ag material are laminated on transparent electrodes 4a and 5a, respectively.

Back substrate 9 has the following elements: address electrodes 11, made of Ag material, formed on one principal surface of back-side glass substrate 10; dielectric layer 12 for covering address electrodes 11; barrier ribs 13 formed on dielectric layer 12 at positions corresponding to clearances between address electrodes 11; and phosphor layers 14R, 14G, and 14B between barrier ribs 13.

Front substrate 2 faces back substrate 9 with barrier ribs 13 sandwiched so that display electrodes 6 are orthogonal to address electrodes 11, and the outer periphery of the image display region is sealed by a sealing member. Discharge spaces 15 formed between front substrate 2 and back substrate 9 are filled with discharge gas such as Ne—Xe 5% at pressure of 66.5 kPa (500 Torr).

Crossing parts between display electrodes 6 and address electrodes 11 in discharge spaces 15 work as discharge cells 16 (unit light emitting regions).

As front-side glass substrate 3 and back-side glass substrate 10, glass substrates that are easily increased in area, have high flatness, are inexpensive, and are manufactured by a float method are used.

In the structure discussed above, bus electrodes 4b and 5b on front-side glass substrate 3 are formed of Ag electrodes. If front-side glass substrate 3 contains Sn<sup>++</sup>, the glass substrate yellows even when each of transparent electrodes 4a and 5a is interposed between each of bus electrodes 4b and 5b and glass substrate 3. Depending on the degree of the yellowing, an image display characteristic of the image display device is adversely affected.

The glass substrate used as front-side glass substrate 3 of PDP 1 is analyzed to determine Sn<sup>++</sup> content on the surface thereof on which bus electrodes 4b and 5b containing Ag are

to be formed. When the appearance quality is concerned, back-side glass substrate 10 is also analyzed to determine Sn<sup>++</sup> content thereof on the surface on which address electrodes 11 containing Ag are to be formed.

Specifically, reflectance of the glass substrate at the wavelength of 220 nm is measured, and the analysis is performed based on the reflectance. This method is provided based on inventors' study. The inventors found the following facts:

the reflectance near the wavelength of 220 nm increases with increase in Sn<sup>++</sup> content on the glass substrate; and there is a correlation between the reflectance near the wavelength of 220 nm and coloring of the glass substrate by silver colloid.

Here, the reflectance may be measured by a general measuring device.

The Sn<sup>++</sup> content on the glass substrate is determined by a secondary ion-mass spectrometry (SIMS) or an inductively-coupled plasma (ICP) optical emission spectrometry. An allowance of Sn<sup>++</sup> content is determined based on a calibration curve derived from the relation between the Sn<sup>++</sup> content determined by the spectrometry and the measured reflectance. The allowance of Sn<sup>++</sup> content can be therefore determined from the reflectance without breaking the glass substrate.

In other words, firstly, the surface on the non-contact side with tin (top surface) of the glass substrate manufactured by the float method is uniformly removed by thickness of 3, 7, 15, or 20  $\mu\text{m}$ , and reflection spectrum of the remaining glass substrate is measured at wavelength of 200 to 300 nm. The measurement result is shown in FIG. 2. FIG. 2 also shows a measurement result of a glass substrate without removal for comparison. The reason why the top side surface is removed is as follows. Adhesion and diffusion amounts of tin are less and hence the yellowing degree is lower on the top-side surface than the bottom-side surface (contact side with tin), so that a bus electrode made of Ag material is generally formed on the top-side surface. When the Ag electrode is formed on the bottom side, the coloring degree is two or three times higher than that in the case that the Ag electrode is formed on the top side.

FIG. 2 shows that, when removed thickness is 15  $\mu\text{m}$  or less, reflectance at peak A near the wavelength of 220 nm decreases with increase of the removed thickness. When removed thickness is 15  $\mu\text{m}$  or more, the decrease of the reflectance stops. It is considered that Sn<sup>++</sup> content monotonously decreases in the depth direction from the top side of the glass substrate. The result shown in FIG. 2 matches with the consideration, and hence the decrease of the reflectance at peak A is considered to match with the decrease of Sn<sup>++</sup> content.

Next, for clarifying a relation between the peak near the wavelength of 220 nm appearing in the reflection spectrum and yellowing of the glass substrate, an Ag electrode is formed on the glass substrate and coloring degree of the glass substrate is measured. In other words, 5  $\mu\text{m}$  thick silver paste as the Ag electrode is applied onto the glass substrate by screen printing, they are calcined at 600°C., and a relation between the coloring degree of the glass substrate and reflectance at the wavelength of 220 nm is investigated. FIG. 3 shows the investigation result. The coloring degree of the glass substrate is evaluated using b\* in a L\*a\*b\* color system (JIS Z 8729). The larger b\* value is, the higher the degree of yellowing is. The coloring degree of the glass substrate is measured from the side having no Ag electrode. As shown in FIG. 3, the reflectance of light at the wavelength of 220 nm on the glass substrate and the coloring degree b\* of the glass substrate are directly proportional.

The investigation result discussed above shows that increase of the reflectance of the glass substrate at the wavelength of 220 nm has a correlation to the Sn<sup>++</sup> content in the glass substrate, namely content of reducing material at least causing yellowing. Therefore, by measuring the reflectance at the wavelength of 220 nm, the Sn<sup>++</sup> content in the glass substrate on which the Ag electrode is to be formed can be analyzed based on the calibration curve, and the degree of yellowing of the glass substrate can be also estimated. This method is useful for evaluating whether or not a selected glass substrate is optimum for an image display device.

In FIG. 2, after 15  $\mu\text{m}$  or more thick glass substrate is removed, the reflectance (about 2%) near the wavelength of 220 nm is not resulted from existence of Sn<sup>++</sup> but by bottom part of a reflection spectrum having a peak at another wavelength. The stop of the decrease of the reflectance at the wavelength of 220 nm is considered to be caused by decrease of the Sn<sup>++</sup> content in the glass substrate. FIG. 4 shows difference  $\Delta R(\lambda)=R_S(\lambda)-R_B(\lambda)$ . Here,  $R_S(\lambda)$  is a reflection spectrum of the glass substrate shown in FIG. 2, and  $R_B(\lambda)$  is a reflection spectrum in a nonexistent state of Sn<sup>++</sup>, namely in a state where the removal of 15  $\mu\text{m}$  or more thick glass substrate stops the decrease of the reflectance. Reflection difference  $\Delta R$  is considered to indicate the existence of Sn<sup>++</sup>.

The reflectance at the wavelength of 220 nm may be read from a reflection spectrum distribution as shown in FIG. 2. However, for more precisely evaluating signal strength of the reflection spectrum having a correlation to Sn<sup>++</sup>, the following method can be used. Reflection spectrum is measured in a wider range of wavelength, for example 180 to 280 nm. The measured reflection spectrum is then divided into two Gaussian peaks of a component having a correlation to Sn<sup>++</sup> and a component having no correlation to Sn<sup>++</sup> shown in FIG. 5 by a curve fitting method using a following equation 1. Then, areas of the components with Gaussian peak having a correlation on Sn<sup>++</sup> are compared with each other to evaluate.

$$M1 \exp\left\{-\frac{(1240/\lambda - 1240/M2)^2}{M3^2}\right\} + \quad (Eq. 1)$$

$$M4 \exp\left\{-\frac{(1240/\lambda - 1240/M5)^2}{M6^2}\right\}.$$

Where,  $\lambda$  is a wavelength (nm), and M1 to M6 are fitting parameters.

The lower limit of the measured wavelength range is set at 180 nm because oxygen in atmospheric air absorbs light at a wavelength lower than 180 nm, hence vacuum or atmosphere containing no oxygen is required for measurement, and construction of a measuring system and measurement require much effort.

This method is also useful for evaluating whether or not a selected glass substrate is optimum for an image display device.

The position of the wavelength of the peak of the reflectance caused by Sn<sup>++</sup> can slightly change depending on the manufacturing condition and the composition of the glass substrate. Therefore, for increasing analysis accuracy of Sn<sup>++</sup>, it is more effective to analyze not only the reflectance at wavelength of 220 nm but also the bottom part of the reflectance extending to wider wavelength range, for example 200 to 250 nm.

Specifically, wavelength  $\lambda^*$  maximizing difference  $\Delta R(\lambda)=R_S(\lambda)-R_B(\lambda)$  in a wavelength range of 200 to 250 nm is considered to indicate the existence of Sn<sup>++</sup>, as shown in FIG.

6. Here,  $R_S(\lambda)$  is a reflection spectrum of the glass substrate, and  $R_B(\lambda)$  is a reflection spectrum in a nonexistent state of Sn<sup>++</sup>. In FIG. 6, wavelength  $\lambda^*$  maximizing  $\Delta R(\lambda)$  is additionally written in FIG. 4. Sn<sup>++</sup> content in the glass substrate is analyzed based on the reflectance  $R_S(\lambda^*)$  at wavelength  $\lambda^*$  or reflectance difference  $\Delta R(\lambda^*)=R_S(\lambda^*)-R_B(\lambda^*)$ .

The reflectance difference  $\Delta R(\lambda^*)=R_S(\lambda^*)-R_B(\lambda^*)$  means the maximum value of  $\Delta R(\lambda)=R_S(\lambda)-R_B(\lambda)$ . Here,  $R_S(\lambda)$  is a reflection spectrum of the glass substrate at wavelength of 200 to 250 nm, and  $R_B(\lambda)$  is a reflection spectrum in a nonexistent state of Sn<sup>++</sup>.

10 Sn<sup>++</sup> locally exists only in a region from the outermost surface of the glass substrate to depth of about 15  $\mu\text{m}$ , as shown in FIG. 2. Therefore, reflection spectrum on the glass substrate of which top part having thickness of 15  $\mu\text{m}$  or more, preferably 20  $\mu\text{m}$  or more, is removed can be set as reflection spectrum  $R_B(\lambda)$  in the nonexistent state of Sn<sup>++</sup>.

15 Another specific method of analyzing reflection spectrum also including the extending bottom part of the reflection spectrum is provided as follows. A mean reflectance is determined from area integral of reflection spectrum at the wavelength of 200 to 250 nm, for example, and Sn<sup>++</sup> content is analyzed.

20 Either of the methods discussed above is useful for evaluating whether or not a selected glass substrate is optimum for an image display device.

25 A judgment standard for the analysis result of the Sn<sup>++</sup> content on the surface of the glass substrate on which the Ag electrode is to be formed is described hereinafter.

30 Existence of Sn<sup>++</sup> reduces Ag<sup>+</sup> of the Ag electrode to generate Ag colloid, and the glass substrate yellows. The coloring (yellowing) degree of the glass substrate is determined based on the Sn<sup>++</sup> content, so that an allowance of the Sn<sup>++</sup> content is a judgment standard when the glass substrate is used for an image display device.

35 As shown in the result of FIG. 2, for preventing the yellowing, it is preferable that the following parameter is smaller:

reflectance at a wavelength indicating existence of Sn<sup>++</sup>, such as reflectance  $R_S(220)$  at the wavelength of 220 nm; reflectance  $R_S(\lambda^*)$  at wavelength  $\lambda^*$  maximizing reflection spectrum difference  $\Delta R(\lambda)=R_S(\lambda)-R_B(\lambda)$ ; reflectance difference  $\Delta R(\lambda^*)=R_S(\lambda^*)-R_B(\lambda^*)$ ; or mean reflectance  $R_{S-mean}(200-250)$  at wavelength of 200 to 250 nm. Specifically, reflectance  $R_S(220)$  is 5% or less, reflectance  $R_S(\lambda^*)$  is 5% or less, reflectance difference  $\Delta R(\lambda^*)$  is 3% or less, or mean reflectance  $R_{S-mean}(200-250)$  is 5% or less. In this case, it is verified that the Sn<sup>++</sup> content is so low that the yellowing of the glass substrate presents no problem even when an image display device is manufactured by forming an Ag electrode on the glass substrate.

40 However, the low Sn<sup>++</sup> content in the glass substrate can be caused by weak reducing force of the atmosphere in a float furnace. In this case, disadvantageously, metallic tin in a tin bath continuously oxidizes and volatilizes in manufacturing the glass substrate. Too low Sn<sup>++</sup> content in the glass substrate is not preferable in manufacturing the glass substrate.

45 It is therefore preferable that reflectance  $R_S(220)$  is between 2.5% and 5%, reflectance  $R_S(\lambda^*)$  is between 2.5% and 5%, reflectance difference  $\Delta R(\lambda^*)$  is between 0.5% and 3%, or mean reflectance  $R_{S-mean}(200-250)$  is between 2.5% and 5%.

50 When a measured reflectance of the glass substrate exceeds the range discussed above, Sn<sup>++</sup> content exceeds an allowance where yellowing of the glass substrate is prevented from affecting the image display. In this case, when an image

display device is manufactured by forming an Ag electrode on the glass substrate, yellowing producing a defect in the image display device occurs.

When the  $\text{Sn}^{++}$  content is determined to exceed the allowance, the reducing force in a float furnace is weakened in manufacturing the glass substrate, and the  $\text{Sn}^{++}$  content of the glass substrate is decreased. For weakening the reducing force in the float furnace, specially, hydrogen concentration in the float furnace is decreased. Mixed gas of hydrogen and nitrogen is generally used as atmospheric gas in the float furnace. The mixed gas contains 2 to 10 vol % of hydrogen. The reducing force is controlled by changing hydrogen concentration in this hydrogen concentration range in response to the allowance of the  $\text{Sn}^{++}$  content.

FIG. 7 shows a manufacturing apparatus of the glass substrate. A manufacturing method of the glass substrate is described.

Material for the glass substrate is injected into melting furnace 21, heated to a high temperature to be molten, and then supplied to float furnace 22. Float furnace 22 has molten tin 24 in its lower part, and has reducing atmosphere 25 (mixed gas of hydrogen and nitrogen) for preventing oxidation of tin in its upper space. Molten glass is continuously moved on molten tin 24 and molded as plate-like glass ribbon 23. Glass ribbon 23 is lifted up from the tin bath and moved to slow cooling furnace 27 by conveying roller 26. Distortion occurring during the molding is decreased by slowly cooling glass ribbon 23 in slow cooling furnace 27.

After the slow cooling process, a surface analyzing process of measuring reflectance with reflectance measuring device 32 and analyzing the  $\text{Sn}^{++}$  content of the glass substrate is performed in the manufacturing apparatus in FIG. 7. Reflectance measuring device 32 measures the following parameter:

reflectance at a wavelength indicating existence of  $\text{Sn}^{++}$  in the glass substrate, such as reflectance  $R_S$  (220) at the wavelength of 220 nm;

reflectance  $R_S(\lambda^*)$  at wavelength  $\lambda^*$  maximizing  $\Delta R(\lambda) = R_S(\lambda) - R_B(\lambda)$ ;

reflectance difference  $\Delta R(\lambda^*) = R_S(\lambda^*) - R_B(\lambda^*)$ ; or

mean reflectance  $R_{S-mean}$  (200-250) at wavelength of 200 to 250 nm.

When the  $\text{Sn}^{++}$  content is determined to exceed the allowance based on the measured reflectance, concentration of the atmosphere gas is controlled to weaken the reducing force in float furnace 22. For preventing yellowing, it is preferable that the reflectance is as low as possible. While, when the reducing force of atmosphere 25 in float furnace 22 is excessively weakened for reducing the  $\text{Sn}^{++}$  content in the glass substrate, disadvantageously, metallic tin contained in molten tin 24 continuously oxidizes and volatilizes in manufacturing the glass substrate.

Therefore, when the reflectance corresponding to the  $\text{Sn}^{++}$  content in the glass substrate is higher than the allowance value discussed above, the hydrogen concentration of the atmosphere in the float furnace is controlled to be decreased. When the reflectance is lower than the allowance value, the hydrogen concentration is preferably increased for preventing oxidation of the metallic tin.

This reflectance measurement can be performed nondestructively, in a non-contact matter, and in a short time, so that the measurement is applicable also to a process control of a routine manufacturing process of a glass substrate. The image display device is especially required to be uniform on its surface, so that the reflectance is preferably measured at a plurality of positions for recognizing dispersion on the glass substrate.

The  $\text{Sn}^{++}$  content can be evaluated by the secondary ion-mass spectrometry (SIMS) or the inductively-coupled plasma (ICP) optical emission spectrometry. However, these methods are destructive inspections and can hardly be used for measurement on a large area, so that the methods are inappropriate for in-line measurement of  $\text{Sn}^{++}$  content in a glass substrate in the glass substrate manufacturing process. When  $\text{Sn}^{++}$  content in a predetermined sample is measured, reflectance of the sample is measured, and a calibration curve is prepared, however,  $\text{Sn}^{++}$  content can be determined based on the reflectance.

When hydrogen concentration of the atmosphere in the float furnace increases, reducing property of the atmosphere is increased to increase the  $\text{Sn}^{++}$  content of the glass substrate, and the yellowing of the glass substrate presents a problem, as discussed above. The variation in the  $\text{Sn}^{++}$  content of the glass substrate appears as difference in yellowing degree of the glass substrate, so that this variation must be within a certain range. When the reflectance of the glass substrate is higher than the predetermined range discussed above, the hydrogen concentration in the float furnace is decreased. The decreasing weakens the reducing property of the atmosphere, so that the reflectance of the glass substrate can be decreased.

After the surface analyzing process of measuring reflectance, in a cutting process, glass ribbon 23 is cut into an arbitrary size by a cutter 28 and glass substrate 100 is produced.

Though the reducing force in float furnace 22 is controlled to weaken, the analyzed  $\text{Sn}^{++}$  content of the glass substrate on which an Ag electrode is to be formed sometimes exceeds the allowance. In this case, as shown in FIG. 8, the Ag electrode receiving surface of the glass substrate is partially removed until the  $\text{Sn}^{++}$  content becomes within the allowance in surface removing furnace 29 in a surface removing process. In other words, by controlling the reducing force in float furnace 22 to weaken and partially removing the surface of the glass substrate, the surface of the glass substrate formed so as to have decreased  $\text{Sn}^{++}$  content is further partially removed. In this case, removed thickness can be decreased comparing with the case that the surface is partially removed without controlling the reducing force in float furnace 22. When the reducing force in float furnace 22 is not controlled, as shown in FIG. 2,  $\text{Sn}^{++}$  exists in a range from the glass surface to depth of about 15  $\mu\text{m}$ . For thoroughly removing  $\text{Sn}^{++}$ , the glass substrate having a large area must be uniformly removed by thickness of 15  $\mu\text{m}$  or more, preferably 20  $\mu\text{m}$  or more. This removing process requires mirror finish, and increasing the removed thickness increases cost extremely, so that decrease of the removed thickness is extremely economical.

The surface removing process may employ a chemical method or a physical method. In the chemical method, the glass substrate surface is etched by dipping glass substrate 100 into etchant 30 such as aqueous hydrofluoric acid or aqueous sodium hydroxide. The physical method includes a buffing method or a sand blasting method. Sufficient surface removing thickness is about 3 to 15  $\mu\text{m}$ , as shown by the study of the reflectance.

In a method shown in FIG. 9, surface removal is performed in surface removing furnace 29,  $\text{Sn}^{++}$  content in glass substrate 100 is analyzed again by reflectance measuring device 32 in a second surface analyzing process, and surface removal is performed again if necessary. Thus, the surface analyzing process and the surface removing process are repeated and the surface state of the glass substrate is severely controlled, thereby further increasing the advantage of the present invention.

When the  $\text{Sn}^{++}$  content in the glass substrate is determined to be higher than the allowance, the glass substrate may be used as a back-side glass substrate of an image display device. When the  $\text{Sn}^{++}$  content in the glass substrate is determined to be not higher than the allowance, the glass substrate may be used as a front-side glass substrate of an image display device.

When a PDP is the image display device manufactured using the glass substrate formed as discussed above, the PDP does not generate yellowing that is so strong as to affect the image display characteristic, and can sufficiently display an image.

An investigation result of the PDP manufactured in accordance with the present invention is described.

The surface of a glass substrate (PD-200 manufactured by Asahi Glass Co. Ltd.) manufactured by the float method is partially removed so that various amount of the reducing layer remains on the surface of the glass substrate. In other words, a maximum value of  $\Delta R(\lambda) = R_S(\lambda) - R_B(\lambda)$ , namely difference between reflection spectrum  $R_S(\lambda)$  and reflection spectrum  $R_B(\lambda)$  in a wavelength range of 210 to 250 nm, is 0.1%, 0.8%, 2.1%, 3.3%, or 4.0%. Specifically, surface removal is performed by dipping the glass substrate into etchant composed of aqueous hydrofluoric acid (10%), and the surface removing thickness is controlled using the dipping period. When temperature of the aqueous hydrofluoric acid is set at 27°C, etching speed is 2  $\mu\text{m}/\text{min}$ . After the dipping for a predetermined period, the glass substrate is washed. Then, reflection spectrum is measured.

Using these glass substrates, three kinds of PDPs having different resolution and structure are manufactured, and a relation between reflection spectrum difference  $\Delta R(\lambda)$  and coloring degree ( $b^*$ ) by yellowing of the PDPs is evaluated.

PDP111 corresponds to video graphics array (VGA) (480×640 pixel), and has a transparent electrode between an Ag electrode (bus electrode) and a glass substrate. PDP222 corresponds to extended graphics array (XGA) (768×1024 pixel), and has a transparent electrode between an Ag electrode and a glass substrate. PDP333 corresponds to XGA and has no transparent electrode between an Ag electrode and a glass substrate.

Table 1 shows a measurement result of reflection spectrum difference  $\Delta R(\lambda)$  and coloring degree ( $b^*$ ) by yellowing of three kinds of PDPs. The value of  $b^*$  is preferably as small as possible, but, actually, the yellowing has no particular problem when  $b^*$  is 2 or smaller. The PDPs have no problem as an image display device in the following conditions:

$\Delta R(\lambda)$  is about 3% or lower in PDP111 having a transparent electrode between the Ag electrode and the glass substrate and a wide pixel interval;

$\Delta R(\lambda)$  is about 2% or lower in PDP222 having a transparent electrode between the Ag electrode and the glass substrate but a narrow pixel interval; and

$\Delta R(\lambda)$  is about 1% or lower in PDP333 having no transparent electrode.

TABLE 1

| 5  | $\Delta R [\%]$ | b *    |        |        |
|----|-----------------|--------|--------|--------|
|    |                 | PDP111 | PDP222 | PDP333 |
| 10 | 0.1             | 0.4    | 0.4    | 0.5    |
|    | 0.8             | 0.8    | 0.6    | 1.3    |
|    | 2.1             | 1.2    | 2.3    | 2.2    |
|    | 3.3             | 2.0    | 2.8    | 4.2    |
|    | 4.0             | 2.4    | 3.4    | 5.5    |

The advantage of the present invention is useful for not only a PDP but also an image display device having the structure where an Ag electrode is formed on a glass substrate having  $\text{Sn}^{++}$  on its surface. This glass substrate is a glass substrate formed by the float method, for example.

#### INDUSTRIAL APPLICABILITY

The present invention provides an image display device that can suppress yellowing from occurring on a glass substrate manufactured by the float method even when an Ag electrode is formed on the glass substrate, and has high image display quality. The present invention provides a manufacturing method of the glass substrate for use in the image display device.

The invention claimed is:

1. An evaluating method of a front-side glass substrate manufactured by a float method for an image display device, the evaluating method comprising:

measuring reflection spectrum at a wavelength of 180 to 280 nm;  
dividing the measured reflection spectrum into two components by a curve fitting method using a following equation (2)

$$M1\exp\left\{-\frac{(1240/\lambda - 1240/M2)^2}{M3^2}\right\} + M4\exp\left\{-\frac{(1240/\lambda - 1240/M5)^2}{M6^2}\right\} \quad (2)$$

one of the components being a component with Gaussian peak at a wavelength of 220 nm and a correlation to  $\text{Sn}^{++}$ , and the other of the components being a component with no correlation to  $\text{Sn}^{++}$ ;

comparing areas of the components with Gaussian peak at a wavelength of 220 nm having a correlation to  $\text{Sn}^{++}$ ;

and  
analyzing  $\text{Sn}^{++}$  content in the front-side glass substrate, wherein  $\lambda$  is a wavelength (nm), and M1 to M6 are fitting parameters.

\* \* \* \* \*